

[54] SPECTRAL SENSITIZATION OF  
PHOTOGRAPHIC LIGHT-SENSITIVE  
EMULSION

[75] Inventors: **Keisuke Shiba; Motohiko Tsubota**,  
both of Minami-Ashigara, Japan

[73] Assignee: **Fuji Photo Film Co., Ltd.**, Minami-  
Ashigara, Japan

[22] Filed: **Mar. 30, 1973**

[21] Appl. No.: **346,386**

**Related U.S. Application Data**

[63] Continuation of Ser. No. 111,501, Feb. 1, 1971,  
abandoned.

[30] **Foreign Application Priority Data**

Jan. 30, 1970 Japan ..... 45-8231

[52] U.S. Cl. ..... 96/127; 96/130; 96/132;  
96/137; 96/140

[51] Int. Cl. ..... G03c 1/10; G03c 1/18

[58] **Field of Search** ..... 96/120, 127, 130, 140,  
96/137, 132

[56] **References Cited**  
UNITED STATES PATENTS

2,519,001 8/1950 Sprague ..... 96/140  
3,469,987 9/1969 Owens et al ..... 96/120

*Primary Examiner*—J. Travis Brown  
*Attorney, Agent, or Firm*—Sughrue, Rothwell, Mion,  
Zinn & Macpeak

[57] **ABSTRACT**

A method for sensitizing spectrally, a photographic  
sensitive emulsion, which comprises:

- a. dissolving a methine dye containing at least one  
water-soluble group in an organic solvent having a  
water solubility of 10% by weight or less at 35°C,
- b. dispersing the solution in a member selected from  
the group consisting of water and a hydrophilic colloid  
of 2% by weight or less, and
- c. subsequently to the dispersing step, adding the  
dispersion to a light-sensitive emulsion.

28 Claims, 13 Drawing Figures

**FIG. 1****FIG. 2****FIG. 3****FIG. 4****FIG. 5****FIG. 6**

INVENTORS  
KEISUKE SHIBA  
MOTOHIKO TSUBOTA

BY *Sughrue, Rothwell, Mion, Zinn & Macpeak*

ATTORNEYS

**FIG. 7****FIG. 8****FIG. 9****FIG. 10****FIG. 11****FIG. 12****FIG. 13**

SPECTRAL SENSITIZATION OF PHOTOGRAPHIC  
LIGHT-SENSITIVE EMULSION  
CROSS-REFERENCE TO RELATED  
APPLICATIONS

This application is a Continuation Application of our earlier copending Ser. No. 111,501 filed on Feb. 1, 1971, now abandoned, which claims priority from Jan. 30, 1970, based on Japanese Patent Application No. 8231/70.

BACKGROUND OF THE INVENTION

1. Field of the Invention

This invention relates to a method of sensitizing spectrally, a photographic light-sensitive emulsion necessary for the production of photographic light-sensitive materials and more particularly, it is concerned with a method of adding a dye to an emulsion.

2. Description of the Prior Art

It is well known that the technique of spectral sensitization, whereby the light-sensitive wavelength region of a light-sensitive material is sufficiently extended to the visible region, is important for the production of photographic light-sensitive materials and, in particular, is essential for color photographic light-sensitive materials. In general, the step of spectral sensitization resides in dyeing a light-sensitive element dispersed in a photographic light-sensitive emulsion, such as grained silver halide, zinc oxide, cadmium sulfide, titanium oxide, organic silver complexes or organic high molecular weight photoconductors, by the addition of a suitable sensitizing dye. Many efforts have been made with respect to the spectral sensitization of silver halide emulsions. When a sensitizing dye is added to a silver halide emulsion, the adsorption state on the surface of silver halide microcrystals varies markedly with the conditions of said addition, which have a great influence upon photographic properties, such as fogging action, sensitivity, distribution of spectral sensitivity, desensitizing action, stability of sensitivity, and so on. This is disclosed in C. E. K. Mees, "The Theory of the Photographic Process" (1954) 11d Ed., chapter 12, pages 430-500 (McMillan). The most important condition for providing a stable spectral sensitization while keeping a high sensitivity is in fact that every molecule of a sensitizing dye to be added should adsorb soundly on the adsorption site of light-sensitive silver halide crystal without interaction with a binder and without aggregation or deposition in a binder. It also resides in the fact that a sensitizing dye should adsorb uniformly, neither too much nor too little, on every crystal of light-sensitive silver halide dispersed in a light-sensitive emulsion.

Many methods are known for adding sensitizing dyes to light-sensitive emulsions. The most commonly used method consists in dissolving a dye in a water-miscible organic solvent such as acetone, methanol, ethanol, propanol, methyl cellosolve or pyridine and adding the dissolution to an emulsion. Some water may be also added to this organic solvent. See, for instance, French Pat. No. 1,508,489. Furthermore, it may be used as an aqueous solution. The method disclosed in Japanese Patent Publication No. 23,389/69 comprises adding a strong acid to a sensitizing dye having an axochrome of an amidinium ion to thus protonize and then adding the dye in the form of an aqueous solution to the emulsion. The method disclosed in Japanese Patent Publication

No. 22,948/69 comprises dissolving a substantially water-insoluble sensitizing dye in a volatile organic solvent, adding the solution to a hydrophilic colloid and heating the mixture to remove the solvent, thereby dispersing the dye in the hydrophilic colloid. Many devices for dispersing dyes have been proposed; for example, as disclosed in U.S. Pat. No. 3,425,835.

However, these methods have many disadvantages. In the method using a water-miscible organic solvent, 10 the organic solvent used tends to lower the surface activity of a coating agent coexistent to conglomerate an aqueous binder of colloidal character and, in the case of a color photographic light-sensitive material, to briquette a coupler coexistent, so that a high speed coating of, for example, 100 m or more per minute would 15 be very difficult to attain. Furthermore, when added, the organic solvent used is immediately mixed with water and the sensitizing dye adsorbs onto the binder before adsorbing on the silver halide crystal, or it aggregates by itself, so that only a weak spectral sensitization is provided. The method of adding in the form of an aqueous solution has a disadvantage that, in general, the sensitizing dye tends to be decomposed. The method mentioned above with reference to Japanese 20 Patent Publication No. 22,948/69 may somewhat improve the above-mentioned disadvantages but cannot avoid important disadvantages. A first disadvantage is that, since a substantially water-insoluble sensitizing dye is dissolved in an organic solvent and then dispersed to a hydrophilic colloid, the transferring or adsorbing speed of the dye molecule to the silver halide microcrystal is slower than that of the common method. Therefore, this method cannot be adapted to any high speed continuous process for making light- 25 sensitive materials with advantage. Another disadvantage is that, in the case of applying a sensitizing dye to a color photo-emulsion containing any coupler, it is adsorbed by the coupler micells, coupler dispersing oil drops and surfactant micells around the oil drops. Accordingly, the transferring or adsorption of the sensitizing dye to the silver halide microcrystal is so hindered 30 that only a weak spectral sensitization is given. A third disadvantage is a poor influence upon a photographic image obtained. The use of a hydrophilic colloid in the case of dispersion means further addition of the oil and hydrophilic colloid to the emulsion, all of which results in an increase in the thickness, which is a bar to thinning of the emulsion layer. Accordingly, it is preferred 35 to decrease the amount of the hydrophilic colloid used to a large extent or to add immediately the dispersion in water to a light-sensitive emulsion.

SUMMARY OF THE INVENTION

It is therefore the principal object of the present invention to provide a method for spectral sensitization whereby the above-mentioned disadvantages encountered when carrying out high-speed coating can be overcome, and the efficiency of the spectral sensitization can be raised with a decrease in fog so as to be adapted to a high-speed continuous process for making a light-sensitive material.

Accordingly, the object of the present invention can be accomplished by employing a sensitizing dye in which at least one water-soluble group, such as carboxyl, sulfo and sulfate groups, is substituted on the dye molecule, and further employing an organic solvent having a water solubility of 10% or less at 35°C. How-

ever, a solvent having a preferably high vapor pressure and containing a hydroxyl or keto group is preferred. Such dye (which may be either a sensitizing dye or a so-called desensitizing dye) is dissolved in the above-mentioned organic solvent considering its quantity required for complete dissolving, at a temperature of at least 35° C., and then dispersed in water or a hydrophilic colloid, the resulting dispersion being added to a photographic light-sensitive emulsion.

A feature of this invention lies in the chemical structure of the dye used or its characteristics; that is, positive introduction of a water-soluble group, preferably, to give a neutral or anionic property in aqueous systems. The water-soluble group applicable is a sulfo group, carboxyl group or sulfate group. A phosphate group may also be employed. Introduction of such water-soluble group can promote remarkably the transferring or adsorption of the dye from oil drops for dispersing the dye to silver halide microcrystals, while overcoming the hindering action of the coexistent substances, such as a hydrophilic binder, as much as or more than those methods commonly employed. Furthermore, surprisingly, the solubility into the organic solvent as defined above is markedly raised, in general, by a factor of 2 to 30 times. This means that the quantity of entrainment of the organic solvent or hydrophilic colloid into an emulsion is markedly reduced as compared with the commonly used method.

Another important feature of the invention lies in dispersing the dye with a markedly reduced amount of hydrophilic colloid or dispersing an oil in which the dye is dissolved without the need for a hydrophilic colloid.

This method, as compared with the prior art, serves to advantage not only in the thinning of an emulsion layer but also in raising remarkably the efficiency of spectral sensitization and decreasing fog, since there is no aggregation of the dye during dispersing and no interaction with a hydrophilic colloid. In this case, the stability of the oil dispersion in which the dye is dissolved does not matter because the addition to a light-sensitive emulsion is carried out substantially immediately after the dispersion. This is very advantageous for the high-speed production of light-sensitive materials.

#### DETAILED DESCRIPTION OF THE INVENTION

Illustrative of the preferable sensitizing dyes according to the present invention are methine dyes disclosed in U.S. Pat. Nos. 2,238,231, 2,493,748, 2,519,001, and 2,912,329; British Pat. Nos. 846,298 and 944,301; German Pat. Nos. 1,163,671, 1,177,481, and 1,072,467; Japanese Patent Publications Nos. 23467/65, 14112/65, 2607/68, 27165/67, 27166/67, 27167/67, 2606/68, 4930/68, 13823/68 and 27164/68; and sensitizing dyes obtained by the synthetic methods disclosed in U.S. Pat. Nos. 3,177,210 and 2,537,880; British Pat. No. 840,223; German Pat. Nos. 929,080, 1,072,765, and 1,028,718; and French Pat. No. 1,359,683. These dyes may be used alone or in admixture. The supersensitization including the combined use of dyes mentioned in Japanese Patent Publications Nos. 4932/68, 4933/68, 4936/68 and 22884/68 can with advantage be adapted for use in the present invention.

The methine dyes used in the examples which follow are shown below:





Dyes for comparison:



The organic solvent used in this invention must have a high dissolving property with respect to the dyes and a good dispersiveness in the form of fine particles in water or a hydrophilic colloid. To this goal, the solubility in water at 35° C should be at most 10% and the vapor pressure should be preferably high. This requirement is satisfied by having a relatively hydrophilic group, such as hydroxyl, ester or keto group, with a hydrophobic aromatic or aliphatic radical. The organic solvents of alcohol ester or ketone type mentioned in Kirk-Othmer, "Encyclopedia of Technology" Vol. 12, pages 654-686, in particular, Table 2, (1954 ed., The Interscience Encyclopedia Co.) are suitable for use in the invention.

Specific examples of the organic solvents which can be employed in the practice of this invention are given as follows without limiting the same:

- A. methylphenylcarbinol
- B. 2-pentanol
- C. diisobutylcarbinol
- D. mesityl oxide
- E. methyl isobutyl ketone
- F. isopropyl acetate
- G. cellosolve acetate
- H. 2-phenoxyethanol

The dye solution using the organic solvent (as a solvent) is then dispersed in water or a hydrophilic colloid of 2% by weight or less. The dye solution is obtained by

heating and stirring, preferably by means of ultrasonic wave. The dispersing is ordinarily carried out in the presence of a surface active agent of the anionic type by mechanical high speed stirring or ultrasonic wave stirring or both. The hydrophilic colloid is gelatin, polyvinylpyrrolidone, its copolymer, cellulose derivative, alginate polymer, polyvinyl alcohol. Preferably, the polymer should contain a sulfo group or carboxyl group. The resulting dye dispersion is added under molten state to a photographic light-sensitive emulsion almost immediately after dispersing.

The light-sensitive emulsion used may be a hydrophilic colloid in which fine crystals of a light-sensitive material such as silver halide, titanium oxide, zinc oxide or cadmium sulfide, is dispersed. Preferably, a gelatino-silver halide such as -silver iodobromide, -silver bromide, -silver chlorobromide, -silver chloride, -silver iodochlorobromide or their mixtures is employed. Chemical aging may with advantage be carried out by any combination of reducing sensitization, sulfur sensitization and noble metal sensitization. In general, it may be applied to any light-sensitive emulsion to which spectral sensitization is required.

To the photographic emulsion spectrally sensitized according to the present invention may be added any additives which are ordinarily used. Illustrative of these are stabilizers, fog inhibitors, chemical sensitizers, hardeners, color formers, coating agents, development precursors, plasticizers and polymers, except for gelatin. A finished emulsion spectrally sensitized according to this invention is coated onto a suitable support, such as cellulose derivative film, polyethylene terephthalate film, baryta paper, paper, resin laminated paper, synthetic paper, glass sheet, plastic film or metallic sheet.

In the method of spectral sensitization according to this invention, the commonly used method or a super-sensitization method may jointly be used. The quantity of addition may be an amount such as ordinarily used for a light-sensitive material, and preferably  $1 \times 10^{-7}$  to  $1 \times 10^{-3}$  mol per one mol of the light-sensitive material.

A better understanding of the present invention will be obtained from the following examples, which are merely illustrative and not limitative of the present invention.

#### EXAMPLE 1

Predetermined amounts of the organic solvent "H" hereinbefore set forth and dye were taken, mixed, heated, held at about 50° C and radiated by ultrasonic wave with agitation. 500 ml of a 2% gelatin solution was held at about 50° C, into which the dye solution was poured with slight agitation. Then, 50 ml of a 5% aqueous solution of sodium alkylbenzenesulfonate was added and dispersed by means of a high-speed rotary mixer to thus obtain a fine dispersion of oil drops. Thus, the dispersions of the dyes (emulsion) 1 to 8 were obtained:

Table 1

| Dye emulsion No | Dye  | Amount $\times 10^{-7}$ g-mol | Organic solvent | Amount (ml) |
|-----------------|------|-------------------------------|-----------------|-------------|
| 1               | I    | 500                           | H               | 100         |
| 2               | II   | 500                           | H               | 100         |
| 3               | III  | 500                           | H               | 100         |
| 4               | IV   | 250                           | H               | 200         |
| 5               | V    | 500                           | H               | 100         |
| 6               | VI   | 500                           | H               | 50          |
| 7               | VII  | 500                           | H               | 100         |
| 8               | VIII | 500                           | H               | 100         |

Similarly, other dispersions of dyes (emulsion) 9 to 15 were obtained using other organic solvents.

Table 2

| Dye emulsion No. | Dye | Amount $\times 10^{-7}$ g-mol | Organic solvent | Amount (ml) |
|------------------|-----|-------------------------------|-----------------|-------------|
| 9                | I   | 500                           | A               | 100         |
| 10               | I   | 500                           | B               | 100         |
| 11               | VII | 500                           | C               | 100         |
| 12               | I   | 500                           | D               | 100         |
| 13               | V   | 500                           | E               | 100         |
| 14               | VII | 500                           | F               | 100         |
| 15               | IV  | 500                           | G               | 50          |

One kg of a silver iodobromide emulsion prepared in the conventional manner was weighed and made molten at about 40° C. 20 ml to 160 ml of the dye emulsions were added thereto directly after dispersing and held at 35° C while stirring, followed by standing. The silver iodobromide emulsion used was a sulfur-gold sensitized emulsion containing about 0.2 mol of silver per 1 kg emulsion and having an iodine content of 4.0 mol % and an average grain size of about 0.5 micron.

#### BRIEF DESCRIPTION OF THE DRAWINGS

The accompanying drawings, FIGS. 1, 2, 3, 4, 5, 6, 7 and 8, indicate the results obtained by measuring the percentage spectral absorption (A) of the emulsions after the passage of one minute, 30 minutes and 75 minutes, after adding to the foregoing silver iodobromide emulsion each of the dye emulsions 1-8 corresponding to an amount of dye of  $8 \times 10^{-5}$  g-mol; for example, 104 ml in the case of the dye emulsion 1, per one kg of the silver iodobromide emulsion, followed by stirring at 35° C. In the figures, the results after one minute are shown by a dotted curve, the results after 30 minutes are shown by a broken curve, and the results after 75 minutes are shown by a real curve.

FIG. 9 shows the percentage spectral adsorption (A) obtained by adding 80 ml of a solution of dye III in methanol having a molar concentration of  $1 \times 10^{-3}$  per kg of the same emulsion. FIG. 10 shows similarly, the percentage spectral adsorption obtained by the use of dye IV. The features of the spectral sensitization according to the present invention, namely, that the dye is transferred, adsorbed and stabilized on silver halide crystal more rapidly after its addition, will apparently be understood from FIGS. 1-8. Particularly, comparisons with FIG. 3 and FIG. 9, and FIG. 4 and FIG. 10.

#### EXAMPLE 2

One kg of the same silver iodobromide emulsion as that of Example 1 was weighed, made molten and spectrally sensitized by the use of the dye emulsion 4. The emulsion 15 was emulsified under the same conditions as in the emulsion 4 except that water was used in place of the 2% gelatin. The organic solvent G was used in place of H and was directly added to one kg of the above-mentioned emulsion and spectrally sensitized. Furthermore, the same emulsion was spectrally sensitized by the use of a methanolic solution of the dye IV of  $5 \times 10^{-4}$  mol. A hardener and coating agent was added to the emulsions, which were coated onto films to obtain film samples spectrally sensitized.

The thus obtained films were cut and subjected to light wedge exposure using a sensitometer of the S-type made by Fuji Photo Film Co., Ltd. A conversion filter of the David-Gibson type was adapted to a light source having a color temperature of 2666° K to give a color temperature of 5400° K and further, a blue filter of No.

K-31 made by Fuji Photo Film Co., Ltd., was used to give a blue light source, while a minus blue light source was obtained using a yellow filter of No. K-12 made by Fuji Photo Film Co., Ltd. Using these light sources, light wedge exposures of blue and minus blue were carried out.

The exposed films were then developed for 10 minutes and fixed, and their density was measured by means of an S-type densitometer to obtain a blue filter sensitivity (S<sub>b</sub>), yellow filter sensitivity (S<sub>y</sub>) and fog. The results are shown in Table 3.

| Composition of Developer Used |                    |
|-------------------------------|--------------------|
| Water (50° C)                 | 750 ml             |
| Metol                         | 2 g                |
| Anhydrous sodium sulfite      | 100 g              |
| Hydroquinone                  | 5 g                |
| Borax                         | 2 g                |
| Water to 1000 ml              |                    |
|                               | (pH = 8.70 ± 0.10) |

Table 3

| Test No. | Dye | Addition Method          |  | Corresponding amount × 10 <sup>-7</sup> g-mol | Photographic Characteristics |                |         |
|----------|-----|--------------------------|--|-----------------------------------------------|------------------------------|----------------|---------|
|          |     | Solvent mol              |  |                                               | S <sub>y</sub>               | S <sub>b</sub> | Fog     |
| 1        | —   | —                        |  | 0                                             | —                            | 100            | 0.10    |
| 2        | IV  | methanol                 |  | 5                                             | 91                           | 95             | 0.13    |
| 3        |     | 5 × 10 <sup>-4</sup> mol |  | 10                                            | 100                          | 83             | 0.13    |
| 4        |     |                          |  | 20                                            | 100                          | 71             | 0.13*   |
| 5        |     |                          |  | 40                                            | 100                          | 39             | 0.18    |
| 6        | IV  | Emulsion 4               |  | 6.7                                           | 100                          | 90             | 0.10    |
| 7        |     |                          |  | 1.3                                           | 110                          | 75             | 0.09    |
| 8        |     |                          |  | 2.6                                           | 140                          | 57             | 0.10**  |
| 9        |     |                          |  | 5.2                                           | 91                           | 32             | 0.11    |
| 10       | IV  | Emulsion 15              |  | 6.7                                           | 105                          | 90             | 0.10    |
| 11       |     |                          |  | 1.3                                           | 125                          | 70             | 0.09    |
| 12       |     |                          |  | 2.6                                           | 160                          | 45             | 0.09*** |
| 13       |     |                          |  | 5.2                                           | 80                           | 25             | 0.09    |

\*Same sample as spectrogram of FIG. 11

\*\* Same sample as spectrogram of FIG. 12

\*\*\*Same sample as spectrogram of FIG. 13

The features and advantages of the present invention will be understood from these results.

Although the present invention has been adequately described in the foregoing specification and examples included therein, it is readily apparent that various changes and modifications may be made without departing from the scope thereof.

To reiterate, the present invention is directed to a method for sensitizing spectrally a photographic sensitive emulsion, which comprises dissolving a methine sensitizing dye containing at least one water-soluble group in the organic solvent, having a water solubility of 10% by weight or less at 35° C, dispersing the solution in a member selected from the group consisting of water and a hydrophilic colloid of 2% by weight or less, and subsequently to the dispersing step, adding the dispersion to a light-sensitive emulsion.

The term "high vapor pressure" as pertaining to the organic solvent applicable to the present invention is directed to an organic solvent which is preferably volatile at room temperature and more preferably, an organic solvent having a vapor pressure of more than 50 mm hg at 20° C so that the solvent can be readily removed from the emulsion layer in the course of the drying process after coating the emulsion onto the support.

As to the organic solvents applicable to the present invention, other than those already enumerated, reference is made to Kirk-Othmer, "Encyclopedia of Technology," Vol. 12, pages 654-686.

With regard to the hydrophilic colloids applicable to the present invention, applicants wish to point out that in addition to those already enumerated in the specification, polyacrylic acid polymers, maleic anhydride polymers, polyvinylbenzenesulfonate, and the like are equally applicable. Also, it is to be pointed out that the terms "polyvinylpyrrolidone" and "polyvinyl alcohol" as used in the specification regarding the hydrophilic colloids applicable, pertain to polymers and copolymers of these compounds. As for the molecular weight range of these polymers applicable to the present invention, it may be generally said that they should be within the range of from  $1 \times 10^4$  to  $2 \times 10^5$ .

As for the cellulose derivatives applicable as hydrophilic colloids, there are carboxy methyl cellulose, carboxy ethyl cellulose, cellulose alginate, and partially hydrolyzed cellulose alginate. The molecular weight range of the cellulose derivatives should preferably be within  $1 \times 10^4$  to  $2 \times 10^5$ .

20 Regarding the polyvinylpyrrolidone and copolymers

of same, it is preferred that the polyvinylpyrrolidone have a molecular weight range of from  $1 \times 10^4$  to  $1 \times 10^6$ . As for the copolymers, polyvinylpyrrolidone may be copolymerized with acrylic amides or vinyl acetate, 45 the polyvinylpyrrolidone in each being of from 0 to 50% by weight of the acrylic amide. It is also preferred that the polyvinylpyrrolidone copolymers employed have a molecular weight range of from  $1 \times 10^4$  to  $2 \times 10^5$ .

50 In addition to the water-soluble groups applicable to the polymers of the present invention, which have already been enumerated, there are the added groups of thiosulfonate, thiosulfate, ammonium, amino, cyano, hydroxyl, ureido, ethyleneoxide, and the like. These water-soluble groups are applicable equally as well to the methine sensitizing dye employed herein.

What is claimed is:

1. A method for sensitizing spectrally, a photographic light sensitive emulsion, comprising silver halide dispersed in a hydrophilic colloid comprising
  - a. dissolving a methine dye containing at least one water-soluble group in an organic solvent having a water solubility of 10% by weight or less at 35° C,
  - b. dispersing the solution in a member selected from the group consisting of water and a hydrophilic colloid of 2% by weight or less,
  - c. subsequently to the dispersing step, adding the dispersion to the light-sensitive silver halide emulsion.
2. The method of claim 1, wherein said water-soluble

11

group is a member selected from the group consisting of a carboxyl group, a sulfo group, a sulfate group and a phosphate group.

3. The method of claim 1, wherein said methine dye

12

substituted alkyl group of from 1 to 5 carbon atoms as the N-substitute thereof.

4. The method of claim 1, wherein the methine dye is a member selected from the group consisting of:

Br<sup>-</sup>

comprises a cyanine nucleus having a sulfo-containing

and



5. The method of claim 1, wherein at least two methine dyes are used in a supersensitizing combination.

6. The method of claim 1, wherein said organic solvent is a material containing a hydrophilic group and a hydrophobic aromatic or aliphatic radical.

7. The method of claim 6, wherein said hydrophilic group is a member selected from the group consisting of a hydroxyl group, an ester group and a keto group.

8. The method of claim 1, wherein the organic solvent is a member selected from the group consisting of methyl-phenylcarbinol, 2-pentanol, diisobutylcarbinol, mesityl oxide, methyl isobutyl ketone, isopropyl acetate, cellosolve acetate and 2-phenoxyethanol.

9. The method of claim 1, wherein said hydrophilic colloid is a member selected from the group consisting of gelatin, polyvinylpyrrolidone polymer, copolymers of polyvinylpyrrolidone, cellulose derivative, alginic polymer, polyvinyl alcohol, polyacrylic acid polymer, maleic anhydride polymer, and polyvinylbenzenesulfonate polymer.

10. The method of claim 9, wherein the polymer contains a member selected from the group consisting of a sulfo group, a carboxyl group, a thiosulfonate group, a thiosulfate group, an ammonium group, an amino group, a cyano group, a hydroxyl group, a ureido group, and an ethylene oxide group.

11. The method of claim 9, wherein the cellulose derivative is a member selected from the group consisting of carboxymethyl cellulose, carboxyethyl cellulose, cellulose alginate, and partially hydrolyzed cellulose acetate.

12. The method of claim 9, wherein the polyvinylpyrrolidone copolymer is a copolymer of polyvinylpyrrolidone with a member selected from the group consisting of acrylic amide and vinyl acetate.

13. The method of claim 9, wherein the molecular weight range of the polymers employed ranges from  $1 \times 10^4$  to  $2 \times 10^5$ .

14. The method of claim 9, wherein the molecular weight of the cellulose derivatives employed ranges from  $1 \times 10^4$  to  $2 \times 10^5$ .

10 15. The method of claim 9, wherein the molecular weight of the polyvinylpyrrolidone polymer ranges from  $1 \times 10^4$  to  $1 \times 10^6$ .

16. The method of claim 9, wherein the molecular weight of the polyvinylpyrrolidone copolymer ranges from  $1 \times 10^4$  to  $2 \times 10^5$ .

15 17. The method of claim 1, wherein the light-sensitive emulsion is a gelatino silver halide emulsion.

18. The method of claim 1, wherein the amount of a dye present is within the range of from  $1 \times 10^{-7}$  to  $1 \times 10^{-3}$  mol of dye per one mol of the light-sensitive material.

19. A photographic light-sensitive silver halide emulsion spectrally sensitized by the method of claim 1.

20 25. A photographic light-sensitive silver halide element, which comprises a support having thereon at least a layer containing the emulsion of claim 1.

21. The photographic light-sensitive silver halide element of claim 20, wherein said support is selected from the group consisting of polyethylene terephthalate, baryta paper, paper, resin laminated paper, synthetic paper, glass sheet, plastic film, metallic sheet and cellulose derivative film.

22. The method of claim 1, wherein in step b the solution is dispersed in the water.

30 35 23. The method of claim 1, wherein in step b the solution is dispersed in the hydrophilic colloid of 2% by weight or less.

24. The method of claim 1, wherein said water-soluble group is a carboxyl group.

40 25. The method of claim 1, wherein said water-soluble group is a sulfo group.

26. The method of claim 1, wherein said water-soluble group is a sulfate group.

45 27. The method of claim 1, wherein said water-soluble group is a phosphate group.

28. The method of claim 1, wherein the dispersing of step b occurs in the presence of a surface active agent.